

# United States Patent

Farrell et al.

[15]

3,660,081

[45]

May 2, 1972

[54] **METHOD MAKING FERROSILICON ALLOY**

- [72] Inventors: John W. Farrell, North Tonawanda; William D. Forgeng, Niagara Falls, both of N.Y.
- [73] Assignee: Union Carbide Corporation, New York, N.Y.
- [22] Filed: Jan. 26, 1970
- [21] Appl. No.: 5,766

**Related U.S. Application Data**

- [63] Continuation-in-part of Ser. No. 652,884, July 12, 1967, abandoned.
- [52] U.S. Cl. .... 75/129, 75/123 L, 75/125
- [51] Int. Cl. .... C22c 39/44, C22c 39/54
- [58] Field of Search .... 75/125, 129

[56]

**References Cited**

**UNITED STATES PATENTS**

|           |         |               |          |
|-----------|---------|---------------|----------|
| 2,906,653 | 9/1959  | Peras .....   | 75/125 X |
| 3,323,899 | 6/1967  | Forgeng ..... | 75/0.5   |
| 3,350,197 | 10/1967 | Beeton .....  | 75/125 X |

Primary Examiner—L. Dewayne Rutledge

Assistant Examiner—J. E. Legru

Attorney—Paul A. Rose, Frederick J. McCarthy, Jr. and Robert C. Cummings

[57]

**ABSTRACT**

Method for producing tough non-friable, non-disintegrating ferrosilicon by the addition of copper to the ferrosilicon in the molten state and controlling the cooling rate of the resultant casting in accordance with the copper content and the calcium and aluminum contents of the casting.

4 Claims, 1 Drawing Figure



**METHOD MAKING FERROSILICON ALLOY**

This application is a continuation-in-part of Ser. No. 652,884, filed July 12, 1967 now abandoned.

This invention relates to ferrosilicon alloys. More particularly, this invention is related to a method for producing ferrosilicon material which is strong, dense, non-friable, and non-disintegrating.

Ferrosilicon is a material widely used as an addition agent in the steel industry, and is usually produced by smelting a mixture of silica, carbon, and iron-bearing materials to obtain a molten alloy which is cast into shapes which are particulated to obtain the size desired by the customer.

Since ferrosilicon is often transported considerable distances from the point of manufacture to the site of ultimate use, and is commonly stored for long periods and exposed to the elements during storage, it is important that the alloy be tough, non-friable, and non-disintegrating.

These requirements present a substantial challenge since ferrosilicon does not inherently possess the above characteristics.

Various techniques, such as slow cooling of the as produced ferrosilicon castings, have been used to improve the toughness of the material and thus reduce friability. However, the problem of self-disintegration during extended storage still remains.

Very rapid cooling of as-produced ferrosilicon castings has been found to significantly suppress self-disintegration; however, such materials are rendered more friable by this type of treatment.

It is, therefore, an object of the present invention to provide a method for preparing ferrosilicon material which is both non-friable and non-self disintegrating, in addition to being strong and dense.

Other objects will be apparent from the following description and claims taken in conjunction with the drawings which shows a graph illustrating cooling rates in accordance with the present invention.

A method in accordance with the present invention comprises preparing a molten ferrosilicon alloy containing about 38 to 90 percent silicon; admixing a copper-bearing material with the molten ferrosilicon to provide between about 0.10 percent and 0.50 percent, and preferably from 0.15 to 0.30 percent copper in the molten ferrosilicon; casting and solidifying the thus treated alloy; and cooling the solidified alloy at a rate such that the amount of zeta phase ( $Fe_2Si_5$ ) in the final alloy is not more than about 10 percent.

The zeta phase,  $Fe_2Si_5$ , which is normally present in substantial amounts in the ferrosilicon alloys hereinabove noted, has been regarded as a cause of disintegration in ferrosilicon alloys. Zeta phase,  $Fe_2Si_5$ , can be observed and the amount present calculated from polished and etched microscopic sections of the alloy in which  $Fe_2Si_5$  appears as a separate and distinct phase. Very slow cooling of the ferrosilicon alloy castings, as previously mentioned, has been found to cause some transformation of the zeta phase,  $Fe_2Si_5$ , to  $FeSi_2 + Si$ , and a reduction in disintegration to some extent. However, there is still need for further improvement in disintegration characteristics.

It has now been discovered, as part of the present invention, that by adding copper to the ferrosilicon alloy in the manner hereinafter described, that a ferrosilicon alloy which is both non-friable, and essentially non-disintegrating, can be produced even with the use of rather rapid cooling rates.

In the practice of a particular embodiment of the present invention, molten ferrosilicon is prepared, e.g., 50 percent silicon, balance essentially iron, and from about 0.10 to about 0.50 percent, preferably 0.15 to 0.30 percent, copper is incorporated in the melt by the addition of elemental copper, e.g., copper clippings, or copper alloys containing 10 percent or more copper so as to avoid introducing objectionable amounts of undesired elements into the ferrosilicon.

After adding the copper, the molten ferrosilicon is cast and solidified, and the casting is caused to cool at a rate such that the final material contains not more than 10%  $Fe_2Si_5$ .

It is important that the  $Fe_2Si_5$  content of the alloy be not more than about 10 percent; otherwise, no significant benefit is obtained from the copper addition.

It has further been discovered that, in addition to the copper content, the calcium and aluminum contents of a ferrosilicon alloy significantly affect the cooling rate required for providing a material containing not more than about 10%  $Fe_2Si_5$ . Further, the relative proportions of calcium and aluminum in the alloy are significant. That is to say, the presence of a given amount of calcium in a ferrosilicon alloy requires a slower cooling rate as compared to the presence of an equal content of aluminum. The calcium actually has an effect of fivefold as compared to aluminum.

Accordingly, in the 30 of the present invention, the maximum cooling rate which is permissible to obtain a ferrosilicon alloy containing not more than about 10%  $Fe_2Si_5$  is determined through the use of the graph of the drawing by locating the curve on the graph corresponding to the effective calcium-aluminum content of the alloy, the effective calcium-aluminum content being  $\%Ca + \%Al/5$ . This is referred to herein as the "Calcium Equivalent" content. The maximum cooling rate for such alloy is then determined by the intersection of the copper content of the alloy with the previously determined curve for the Calcium Equivalent content of the alloy.

For example, with an alloy containing 0.05% Ca, 0.25% Al and 0.26% Cu, the 5 Equivalent content 2 + 0.1% and the maximum cooling rate is 7° C/min. between 850° and 700° 10% illustrated in the drawing at A. It can be stated more generally that for any given copper content, the cooling rate should be to the left of the curve of the drawing corresponding to the Calcium Equivalent content of the alloy.

The casting cooling rates determined in the foregoing manner have been found to ensure substantially complete transformation of zeta phase  $Fe_2Si_5$  to  $FeSi_2 + Si$ . That is to say, the final alloy contains practically no  $Fe_2Si_5$ , and in any event, not more than 10%  $Fe_2Si_5$ .

Maximum cooling rates for various other copper-containing ferrosilicon alloys in order to achieve this condition are shown in Table I and maximum cooling rates for Calcium Equivalents for other than those specifically illustrated can be obtained by interpolation from the graph of the drawing.

TABLE I

| Copper Content % | Calcium Equivalent Content-% | Maximum Coating Rate in Range of 850°C to 700°C |
|------------------|------------------------------|-------------------------------------------------|
| 50 0.1           | 0.05                         | 1.5° per minute                                 |
| 0.1              | 0.2                          | .75° per minute                                 |
| 0.1              | 0.3                          | 0.4° per minute                                 |
| 0.2              | 0.05                         | 5° per minute                                   |
| 0.2              | 0.2                          | 1.5° per minute                                 |
| 0.2              | 0.3                          | 0.7° per minute                                 |
| 55 0.3           | 0.05                         | 14° per minute                                  |
| 0.3              | 0.2                          | 5° per minute                                   |
| 0.3              | 0.3                          | 1.3° per minute                                 |
| 0.35             | 0.05                         | 24° per minute                                  |
| 0.35             | 0.2                          | 8.5° per minute                                 |
| 0.35             | 0.3                          | 2.25° per minute                                |
| 60 .50           | .05                          | 53° per minute                                  |
| .50              | 0.2                          | 22° per minute                                  |
| .50              | 0.3                          | 7.5° per minute                                 |

65 Copper-containing ferrosilicon prepared in the manner aforescribed is remarkable in that it is both tough, i.e., non-friable, and non-disintegrating.

70 With further reference to the drawing, the graph shown sets forth the maximum desirable cooling rates for copper-containing ferrosilicon alloys containing 38 to 90 percent silicon and the indicated Calcium Equivalent contents. The cooling rates are for the temperature range of about 850° to 700°C. since it has been found that this is the range in which controlled cooling is the most critical to achieve transformation of  $Fe_2Si_5$  in copper-containing ferrosilicon. The cooling rate at tempera-

tures above about 850°C. and below about 700°C. can be as fast (or as slow) as desired.

The following example will further illustrate the present invention.

#### EXAMPLE I

A 65 -pound heat of 50 percent ferrosilicon was prepared from an alloy analyzing 48.3 percent silicon, 0.05 percent calcium, 0.70 percent aluminum, 0.015 percent phosphorous, and 0.06 percent copper. The metal was cast at 1,300°C., in 10 -pound increments, into separate clay-graphite crucibles which had been preheated to 1,000°C. No additions were made to the first crucible and copper additions, as elemental copper, were made to provide copper contents of 0.16 percent, 0.35 percent, 1.04 percent in the metal in the remaining crucibles. Immediately after pouring, all crucibles were buried in sand to produce a very slow cooling rate. After cooling to room temperature, the solidified alloy from each crucible was broken with a hammer and pieces of each sample were exposed to the outdoor atmosphere for 10 days. At this time the base alloy sample containing 0.06 percent copper had begun to crumble and was easily abraded by rubbing pieces of the alloy together. The samples containing 0.16 percent, 0.35 percent, and 1.04 percent copper showed no sign of disintegration and were solid, tough, and abrasion resistant.

#### EXAMPLE II

The procedure of Example I was followed to provide ferrosilicon alloys containing 0.06 percent, 0.15 percent, 0.35 percent, 0.55 percent, 0.80 percent and 1.0 percent copper. After 7 days' exposure to the outdoor atmosphere, the alloy containing 0.06 percent copper had noticeably disintegrated. The other alloys showed no sign of disintegration.

#### EXAMPLE III

The procedure of Example I was followed in preparing ferrosilicon alloys containing (A): 0.008% Ca, 0.22% Al and 0.16% Cu and (B): 0.008% Ca, 0.22% Al and 0.22% Cu.

Castings prepared from both alloys were cooled in the temperature range of 850°C to 700°C at a rate of 4° to 5°C per minute. Alloy (A) contained approximately 25%  $Fe_2Si_5$  while alloy (B) was essentially free of  $Fe_2Si_5$ .

5 It has also been found that with ferrosilicon alloys which contain copper, but in which the  $Fe_2Si_5$  phase has not transformed, e.g., rapidly quenched alloys containing 0.16 percent copper, no significant disintegration tendency is observed although the material is easily abraded.

10 In a further embodiment of the present invention, the copper addition is made to the ferrosilicon alloy by mixing a reducible copper compound such as copper oxide, with a silica-carbon charge. The copper compound is reduced concurrently with the silica, and copper is thereby directly incorporated in the ferrosilicon alloy product.

15 The percentages given herein and in the claims are all by weight, unless specified to the contrary.

What is claimed is:

1. A method for producing an essentially non disintegrating ferrosilicon alloy which comprises preparing a molten ferrosilicon alloy containing from about 38 to 90 percent silicon and minor amounts of calcium and aluminum; admixing a copper-rich material with the molten ferrosilicon to provide in the ferrosilicon alloy a copper content of from about 0.10 to 0.50 percent; casting and solidifying the thus treated alloy; and cooling the solidified alloy at a rate such that the amount of zeta phase,  $Fe_2Si_5$ , in the alloy is less than about 10 percent.

2. A method in accordance with claim 1 wherein between about 0.15 and 0.30 percent copper is provided in the ferrosilicon alloy.

3. A method in accordance with claim 1 wherein, for a given copper content, the solidified copper-containing ferrosilicon is cooled in the range of 850° to 750°C. at a rate which is in the area to the left of the curve shown in the graph of the drawing corresponding to the Calcium Equivalent content of the alloy where the Calcium Equivalent = % Ca + % Al/5.

35 4. A method in accordance with claim 1 wherein the copper-rich material is a copper alloy containing at least about 10 percent copper.

40 \* \* \* \* \*